

[54] HEAT-RESISTING STEEL

[75] Inventor: Yoshihiko Abe, Tokyo, Japan

[73] Assignee: Mitsubishi Seiko Kabushiki Kaisha, Tokyo, Japan

[22] Filed: June 5, 1972

[21] Appl. No.: 259,541

|           |         |               |          |
|-----------|---------|---------------|----------|
| 2,080,001 | 5/1937  | Becket.....   | 75/126 F |
| 2,232,705 | 2/1941  | Hull.....     | 75/12 Y  |
| 2,268,427 | 12/1944 | Schlumpt..... | 75/126 F |
| 2,370,124 | 2/1945  | Charlton..... | 75/126 F |
| 2,801,916 | 8/1957  | Harris.....   | 75/128 T |
| 2,848,323 | 8/1958  | Harris.....   | 75/126 P |

Primary Examiner—Hyland Bizot  
Attorney, Agent, or Firm—Wenderoth, Lind & Ponack

## [30] Foreign Application Priority Data

|               |            |          |
|---------------|------------|----------|
| July 20, 1971 | Japan..... | 46-53592 |
| Mar. 6, 1972  | Japan..... | 47-22245 |

[52] U.S. Cl..... 75/124, 75/125, 75/126 C,  
75/126 R, 75/126 P

[51] Int. Cl..... C22c 39/54

[58] Field of Search.... 75/124, 126 T, 126 P, 126 F

## [56] References Cited

## UNITED STATES PATENTS

1,542,233 6/1925 Girin ..... 75/128 T

## [57] ABSTRACT

A heat-resisting steel with superb heat resistance, and yet with a low coefficient of heat expansion, against such high-temperature environments as above 900°C is obtained by uniformly dispersing 2 – 10 percent by weight of one or more carbonitrides selected from the group of those of titanium, zirconium, niobium, tantalum and vanadium into a steel containing 1 – 30 percent by weight of chromium.

1 Claim, 2 Drawing Figures



FIG. 1



FIG. 2



## HEAT-RESISTING STEEL

### BACKGROUND OF THE INVENTION

The present invention relates to heat-resisting steels, and more particularly to steels with superb heat resistance, and yet with a low coefficient of heat expansion, against such high-temperature environments as above 900°C, especially containing sulphur.

In general, heat-resistivity is an indispensable condition for steels to be used in high-temperature circumstances; and beside great strength and toughness not only against high temperatures, such steels are desired to possess great resistance against various high-temperature atmospheres, and yet with a low coefficient of heat expansion.

### SUMMARY OF THE INVENTION

A principal object of the present invention is to provide a heat-resisting steel which satisfies all of the desirable characteristics abovementioned.

It is another object of the present invention to provide a heat-resisting steel which has a heat-resisting quality comparable to that of the conventional heat-resisting steels and yet has such an excellent resistance to sulphur as not being possessed by the conventional heat-resisting steels.

It is a further object of the present invention to provide a heat-resisting steel which, in comparison with the orthodox ones, is superb in heat resistivity, and particularly so against sulphuric matters, while its coefficient of heat expansion is remarkably small.

Another object of the present invention is to provide a heat-resisting steel whose heat resistivity does not rely on such an expensive element as nickel and which chromium in a considerably small amount in comparison with its amount for the orthodox ones, still being provided with superb heat resistance.

A steel according to the present invention is characterized by a chromium containing steel having specific carbonitrides dispersed therein uniformly and finely beyond certain degree of concentration.

### BRIEF DESCRIPTION OF THE DRAWINGS

These and other objects of the present invention will become more apparent to those skilled in the art when considered in reference to the following detailed description in the light of the accompanying drawings wherein:

FIG. 1 is a photograph showing the microstructure of a steel made according to the present invention in which 4.7 percent by weight titanium carbonitride is dispersed into a steel mainly consisting of, by weight, 24.5 percent chromium, 3.5 percent molybdenum and 1.7 percent silicon; and

FIG. 2 is a diagram showing the tensile strength at 700°C of various steels and also the weight increases due to oxidation when they are exposed in the air for 30 hours at 800°C, whereby the steels are those in which, in to the steels mainly consisting of, by weight, 1.0 percent chromium and 0.25 percent molybdenum, various amounts of such sole or complex carbonitrides as titanium, titanium — niobium or zirconium — vanadium are dispersed.

### DETAILED DESCRIPTION OF INVENTION

In the manufacture of the heat-resisting steels of the present invention, it is necessary, firstly, to add car-

bonitride-forming elements to a molten steel prepared beforehand containing a remarkably excessive amount of carbon in comparison with the amounts of oxygen, nitrogen, and sulphur, so as to cause a preferential reaction between the carbonitride-forming elements and the carbon, and then to uniformly disperse and precipitate the thus-obtained solid carbide together with the nitride, and lastly it is necessary for the resulting dispersed carbonitrides to be stable even though it is subject to high temperatures.

As a carbonitride-forming agent, which achieves such a uniform dispersion and thermostability of the solid carbonitride in the microstructure of the steel, a carbonitride may be named with such a composition of one or more elements selected from among such elements as titanium, zirconium, niobium, tantalum and vanadium.

In these carbonitride dispersing agents, the size, uniformity, and quantity of a dispersant are important factors to determine their characteristics, so it has been confirmed that a preferential nitridation of the boron in the molten steel is desirable for this reason.

From the explanation above, it is easily understandable that the steels which can meet the requirements of the present invention can be manufactured by an industrial mass production system.

FIG. 1 shows a microstructure of an example of the heat-resisting alloy steels according to the present invention which clearly shows the uniform distribution of the carbonitrides in the steel.

The effect of a carbonitride uniformly dispersed in the steel on its quality at high temperatures will be explained in reference to FIG. 2. There are shown in it the variations of the steel's high-temperature-proof strength (at 700°C) and high-temperature oxidation resistance (800°C × 30 hr) in the case of the various carbonitrides composed solely or complexly of titanium, or titanium-niobium, or zirconium-vanadium dispersed in a range of up to 10 percent by weight. Irrespective of the kind of the dispersing carbonitride, the respective characteristic curves can be plotted by an identical curve. However, with the amount of the carbonitride being below 2 percent by weight its contribution toward the heat-resistivity of the steel is almost zero; however, if its content surpasses that value, it sharply increases the heat-resistivity of the steel. In the case of the content of the carbonitride being above 7 percent by weight, its effect remains nearly unchanged, so it is understandable that its preferable content should be limited to less than 10 percent by weight, viewed from the aspects of manufacturing technique and economy.

In this case, the components of the matrix having the dispersion of carbonitrides cannot be ignored. Table I indicates the comparative effects of the components of a matrix of steel having the dispersion of titanium or zirconium carbonitrides in 4 percent by weight or so, particularly the comparative effect of the amount of chromium dispersed in the steel, in terms of vanadium attack resistance and oxidation resistance. As is apparent from Table I, the steels which contain no carbonitride and that in which the carbonitride is dispersed into the matrix belonging to the carbon steel (the sample Nos. 1 - 3) have practically no vanadium attack resistivity (refer to the column of the "V-attack resis-

tance") and a little oxidation resistivity (also refer to "Oxidation resistance,") while the steels according to the present invention (sample Nos. 4 and 5) in which chromium is contained in the matrix clearly show that a high temperatures their resistance to corrosion sharply increases. From this result, it is concluded that in a steel to be made a matrix having the dispersion of a carbonitride, it is essential to add chromium. Thus it can be said that the feature of the present invention lies in making advantage of the synergistic effect on the heat resistivity of the steel of the dispersed particles of carbonitrides and chromium contained in the matrix.

In the steels according to the present invention, their corrosion resistivity at high temperatures are remarkably improved by the existence of one or more such elements contained in the matrix as silicon, molybdenum, boron, copper and aluminum as well as the carbonitride-forming elements such as titanium, zirconium, niobium, tantalum and vanadium. In order to show this fact, in Table 3, there is shown the influence of the chemical compositions of the steel according to the present invention on its oxidation resistivity at high temperatures. In Table 3, the steels belonging to the group of samples marked A are those consisting mainly

Table 1

| Sample No. | Kind | Dispersed carbonitride<br>Amount(weight %) | Main alloy components in the matrix | V-attack resistance<br>(loss in weight;<br>mg/cm <sup>2</sup> /hr) | Oxidation resistance<br>(increase in weight;<br>mg/cm <sup>2</sup> /hr) |
|------------|------|--------------------------------------------|-------------------------------------|--------------------------------------------------------------------|-------------------------------------------------------------------------|
|            |      |                                            |                                     |                                                                    |                                                                         |
| 1          | —    | —                                          | 1.0%Cr-0.25%Mo                      | 195                                                                | 1.01                                                                    |
| 2          | —    | —                                          | —                                   | 240                                                                | 1.30                                                                    |
| 3          | Ti   | 4.6                                        | —                                   | 232                                                                | 0.90                                                                    |
| 4          | Ti   | 4.3                                        | 1.1%Cr                              | 132                                                                | 0.26                                                                    |
| 5          | Zr   | 3.8                                        | 1.0%Cr-0.5%Mo                       | 145                                                                | 0.18                                                                    |

Note: Test condition; V-attack resistance - The test piece is immersed in  $V_2O_5$  at 800°C for 20 hours.  
Oxidation resistance - The test piece is exposed in the air at 800°C for 20 hours.

Then, in reference to Table 2, an explanation will be given on the effect of the quantity of chromium to be added into the steel of the present invention. In reference to steels containing chromium in different amounts ranging 1 to 30 percent by weight having a dispersion of 5 to 6 percent by weight titanium-tantalum carbonitride, their oxidation resistivity and sulphurous-acid-gas-proofness were compared at various temperatures. As a result it was revealed that the synergistic effect of the dispersed carbonitride and the chromium contained in the matrix is displayed only in the presence of chromium in concentration over a certain degree which is determined corresponding to temperature. To say more specifically, it is necessary for the steel to contain 5 percent by weight or more, preferably over 10 percent by weight chromium for 900°C, and over 20 percent by weight preferably over 25% by weight chromium for 1,100°C to endure the effect of the present invention, and it can be understood that if the chromium concentration is ensured so much as that, the steels of the present invention have a phenomenal heat-resistivity.

of 25 percent by weight chromium and 8 percent by weight nickel having a dispersion of the carbonitride of titanium and it is understood that their oxidation resistivity is remarkably improved by the composite addition of molybdenum, boron and aluminum. Then, the steels belonging to the group of samples marked B are those consisting mainly of 18 percent by weight chromium with an addition of one selected from among molybdenum, aluminum and copper with carbonitride-forming element added above the concentrations necessary for the formation of the dispersed particles so that they are also dissolved in the matrix, and they show that their oxidation resistivity is remarkably improved. The steels belonging to the group of samples marked C, which consists principally of chromium, are shown to compare the effect of the addition of the elements abovesaid with the effect of addition of silicon, and, it is understood that the addition of these elements has the effect to reduce the necessary amount of chromium which is determined by the kind and the temperature of the environment gases, and silicon is especially effective with respect to this point.

Table 2

| Samples | Dispersing amounts<br>of Ti-carbonitride | Amount of<br>chromium<br>in the matrix (%)<br>weight %) | Increase in weight<br>by oxidation (mg/cm <sup>2</sup> ) |                               | Increase in weight<br>by sulphurous acid gas (mg/cm <sup>2</sup> ) |                                         |                                          |
|---------|------------------------------------------|---------------------------------------------------------|----------------------------------------------------------|-------------------------------|--------------------------------------------------------------------|-----------------------------------------|------------------------------------------|
|         |                                          |                                                         | 900°C×10 hr<br>(in the air)                              | 1,100°C×10 hr<br>(in the air) | 800°C×10hr<br>(in 100%SO <sub>2</sub> )                            | 910°C×10hr<br>(in 100%SO <sub>2</sub> ) | 1,000°C×5hr<br>(in 100%SO <sub>2</sub> ) |
|         |                                          |                                                         |                                                          |                               |                                                                    |                                         |                                          |
| 6.3     |                                          | 1.0                                                     | 34.7                                                     | 274                           | 29.8                                                               | 376                                     | 700<                                     |
| 5.8     |                                          | 2.5                                                     | 36.2                                                     | 312                           | 29.3                                                               | 418                                     | 700<                                     |
| 5.1     |                                          | 5.0                                                     | 0.9                                                      | 295                           | 2.5                                                                | 281                                     | 700<                                     |
| 6.4     |                                          | 10.1                                                    | 0.2                                                      | 212                           | 1.3                                                                | 5.2                                     | 456                                      |
| 5.5     |                                          | 15.0                                                    | 0.0                                                      | 15.4                          | 0.6                                                                | 1.2                                     | 7.8                                      |
| 6.3     |                                          | 20.3                                                    | 0.0                                                      | 9.6                           | 0.0                                                                | 0.3                                     | 1.7                                      |
| 5.7     |                                          | 25.0                                                    | 0.0                                                      | 5.0                           | 0.0                                                                | 0.0                                     | 0.0                                      |
| 5.3     |                                          | 29.7                                                    | 0.0                                                      | 2.2                           | 0.0                                                                | 0.0                                     | 0.0                                      |

Table 3

| Sample mark | Dispersed particle | Chemical composition |      |     |     |     |     |    |     | Oxidation resistance                    |        |        |        |        |
|-------------|--------------------|----------------------|------|-----|-----|-----|-----|----|-----|-----------------------------------------|--------|--------|--------|--------|
|             |                    | Matrix (%)           |      |     |     |     |     |    |     | Oxidation rate (mg/cm <sup>2</sup> /hr) |        |        |        |        |
|             |                    | Kind                 | %    | Cr  | Ni  | Si  | Mo  | Al | Cu  | B                                       | others | 1200°C | 1100°C | 1000°C |
| A           | 1 Ti               | 4.5                  | 25.2 | 8.3 | —   | —   | —   | —  | —   | 0.015                                   | —      | 10.8   | 2.52   | 0.13   |
|             | 2 Ti               | 5.0                  | 25.5 | 8.0 | —   | 2.1 | —   | —  | —   | —                                       | —      | 1.0    | 0.22   | 0.04   |
|             | 3 Ti               | 4.1                  | 25.4 | 8.5 | —   | 2.0 | 1.0 | —  | —   | —                                       | —      | 0.4    | 0.10   | 0.04   |
|             | 1 Ti               | 5.0                  | 18.1 | —   | —   | —   | —   | —  | —   | —                                       | —      | —      | 1.31   | 1.05   |
| B           | 2 Ti+Nb            | 6.7                  | 18.3 | —   | —   | —   | —   | —  | —   | —                                       | Nb     | —      | 1.05   | 0.42   |
|             | 3 Zr               | 5.4                  | 17.6 | —   | —   | 3.8 | —   | —  | —   | —                                       | Zr     | —      | 0.20   | 0.057  |
|             | 4 Ti+Ta            | 3.8                  | 17.3 | —   | —   | —   | —   | —  | 1.3 | —                                       | Ta     | —      | 0.03   | 0.030  |
|             | 5 Ti+V             | 4.3                  | 18.1 | —   | —   | —   | 1.9 | —  | —   | —                                       | V      | —      | 0.15   | 0.082  |
|             | 1 Ti               | 4.5                  | 26.9 | —   | —   | —   | —   | —  | —   | —                                       | Ti     | —      | 0.52   | 0.17   |
|             | 2 Ti               | 4.3                  | 24.5 | —   | —   | —   | —   | —  | —   | —                                       | Ti     | 0.8    | 0.35   | 0.17   |
| C           | 3 Ti               | 4.1                  | 20.0 | —   | —   | 4.2 | —   | —  | —   | —                                       | Ti     | —      | 0.20   | 0.10   |
|             | 4 Ti               | 3.8                  | 18.2 | —   | 1.1 | 3.1 | —   | —  | —   | —                                       | Ti     | —      | 0.27   | 0.10   |
|             | 5 Ti               | 3.2                  | 10.4 | —   | 2.1 | 2.1 | —   | —  | —   | —                                       | Ti     | 1.0    | 0.18   | 0.09   |
|             | 6 Ti               | 4.1                  | 18.0 | —   | 1.7 | —   | 1.0 | —  | —   | 1.0                                     | Ti     | 0.32   | 0.12   | 0.07   |

In this connection, it will be appreciated that the kinds of the additional elements vary depending on the objects of use of the steels, and, in the case where the high strength at high temperatures is not so much needed, even steels in which ferrite constitutes its matrix can do well, and as for the amounts of the elements to be added into the steel, when, at relatively low temperatures, the total amount is 0.2 percent by weight or more, its effect comes to display. However, as the temperature rises, the total amount needs to increase. When 1,000°C is made the object of the steel's high-heat resistivity, the total amount must be made 8 percent by weight or so as shown in Table 3.

Besides, with high-heat-resisting steels, it is desirable to make its coefficient of heat-expansion small when exposed to a high-temperature environment; however, with the steels of the present invention, since the coefficient of heat-expansion of the carbonitride to be dispersed therein is near half that of the steel of the matrix, the coefficient of heat-expansion of the steel of the present invention, in proportion thereto, is expected to become less in comparison with that of the orthodox steels. Table 4 shows the coefficients of heat-expansion at 25° to 600°C of the steels of the present invention in comparison with that of the orthodox steels, which reveals that with the steel of the present invention, its coefficient of heat expansion is lower than its calculated value predictable on the basis of the volume ratio of the matrix and the dispersed particles. That is, in the steels according to the present invention, the dispersed particles having a low coefficient of heat expansion control

even the coefficient of heat expansion of the matrix and bring about an additional advantage that the overall coefficients of heat expansion of the steels are made further smaller than the calculated values.

Though the case where only chromium constitutes the principal alloy element of the matrix has been explained above, such an alloy steel is poor in toughness at a room temperature and yet has not so high strength at a high temperature as compatible with the excellent resistivity to corrosion at high temperatures as stated above. Therefore, when a steel is required also to possess these qualities, the matrix is preferable to be made to be austenite dome with at least one element selected from the group of nickel and manganese, and, also it is effective that the matrix is made with at least one element selected from the group of silicon and molybdenum. Tables 5 and 6 show the effect of the above elements on strength at high temperatures, and Table 7 shows that the steels shown in Table 6 combines an excellent corrosion resistivity at high temperatures with excellent strength at high temperatures. Consequently, in order that the steel according to the present invention secures such high strength at high temperatures in addition to corrosion resistivity at high temperatures as not obtainable in the conventional steels it is required that those elements are added in the same total amount at the maximum as chromium to make the matrix an austenite structure, whereby their maximum amounts in total are 30 percent by weight for the steel containing 30 percent by weight chromium at the maximum.

TABLE 4

| Sample             | Chemical composition (percent) |     |     |      |      |     | Range of the measured temperatures, °C. | Coefficient of heat-expansion |                       |
|--------------------|--------------------------------|-----|-----|------|------|-----|-----------------------------------------|-------------------------------|-----------------------|
|                    | C                              | Si  | Mn  | Ni   | Cr   | Mo  |                                         | Measured value                | Calculated value      |
| Invented steel I   | 0.05                           | 2.1 | 0.5 | —    | 10.4 | 2.1 | (Ti-base) 3.2—                          | 25-600                        | 11.7×10 <sup>-6</sup> |
| Invented steel II  | 0.05                           | 1.7 | 0.6 | —    | 10.7 | 2.2 | (Ti-base) 7.5—                          | 25-600                        | 11.0×10 <sup>-6</sup> |
| Invented steel III | 0.12                           | 1.7 | 0.6 | —    | 24.5 | 8.5 | (Zr-base) 4.7—                          | 25-600                        | 11.0×10 <sup>-6</sup> |
| SUH 3B             | 0.40                           | 2.0 | 0.4 | —    | 11.7 | 1.1 | —                                       | 25-600                        | 12.6×10 <sup>-6</sup> |
| SUH 33B            | 0.17                           | 1.2 | 1.7 | 20.5 | 25.1 | —   | —                                       | 25-600                        | 17.3×10 <sup>-6</sup> |

Table 5

| Composition of matrix | Sample            | Room temperature                                  |                                        |                |                      | High temperature                       |                |                      |
|-----------------------|-------------------|---------------------------------------------------|----------------------------------------|----------------|----------------------|----------------------------------------|----------------|----------------------|
|                       |                   | Kind and amount of dispersed particles (weight %) | Tensile strength (kg/mm <sup>2</sup> ) | Elongation (%) | Reduction of area(%) | Tensile strength (kg/mm <sup>2</sup> ) | Elongation (%) | Reduction of area(%) |
| 10%Cr                 | (Zr + Nb)base 6.2 | 98.6                                              | 8.8                                    | 18.5           | 9.6                  | 41.0                                   | 81.6           |                      |
| 10%Cr + 3%MO          | (Zr + Nb)base 3.5 | 75.4                                              | 21.6                                   | 45.5           | 12.8                 | 69.6                                   | 96.8           | 800                  |
| + 2%Si                | (Ti)base 7.5      | 66.8                                              | 11.8                                   | 22.9           | 10.3                 | 30.3                                   | 75.0           |                      |
| 18%Cr                 | (Ti)base 6.4      | 64.4                                              | 43.2                                   | 60.4           | 22.6                 | 43.4                                   | 64.0           | 800                  |
| 18%Cr + 8%Ni          | (Ti + V)base 4.7  | 70.3                                              | 10.3                                   | 21.0           | 3.4                  | 93.0                                   | 97.9           |                      |
| + 1%Si                | (Ti + V)base 4.5  | 71.5                                              | 41.5                                   | 57.3           | 10.8                 | 78.3                                   | 90.4           | 1,000                |
| 20%Cr                 |                   |                                                   |                                        |                |                      |                                        |                |                      |
| 20%Cr + 20%Ni         |                   |                                                   |                                        |                |                      |                                        |                |                      |

Table 6

| Test Temperatures (°C) | Tensile strength(kg/mm <sup>2</sup> ) |                 |
|------------------------|---------------------------------------|-----------------|
|                        | AISI - 202                            | Invented steel* |
| 800                    | 18.5                                  | 26.0            |
| 900                    | 13.0                                  | 17.7            |
| 1,000                  | 7.5                                   | 9.7             |

\*Note:- AISI-202 + 4.5% by weight of Ti-carbonitride

Table 7

| Atmosphere   |            | Corrosion rate             |                            |
|--------------|------------|----------------------------|----------------------------|
| Kind         | Temp. (°C) | AISI-202                   | Invented steel*            |
| 10% chlorine | 500        | 113g/m <sup>2</sup> /hr    | 118g/m <sup>2</sup> /hr    |
| 90% air      | 1,000      | 1055 do.                   | 445 do.                    |
| Air          | 800        | 0.10mg/cm <sup>2</sup> /hr | 0.04mg/cm <sup>2</sup> /hr |
|              | 900        | 0.32 do.                   | 0.10 do.                   |
|              | 1,000      | 1.6 do.                    | 0.22 do.                   |

\*Note:- AISI-202 + 4.5% by weight of Ti-carbonitride

The following specific examples will serve to illustrate the excellence of the steels according to the present invention in their qualities and an economical advantage as heat-resisting steels.

40

one third of the SUH-33B. Thus, according to the present invention, a heat-resisting steel having better heat resistivities can be obtained quite at a low price.

### EXAMPLE 1

The heat resistivity of the steel according to the present invention which was obtained by dispersing particles of 3.5 percent by weight carbonitride, combined with titanium and niobium in the ratio of 3 : 1, into the steel consisting mainly of, by weight, 20 percent silicon, 10 percent chromium and 3.0 percent molybdenum is shown in Table 8 in comparison with the SUH 33B-steel.

45

Though the so-called 18-8 stainless steel is used in various fields as a heat-resisting stainless steel, the valuable nickel in it was replaced by 5 percent by weight low cost zirconium carbonitride, and the fine particles of the carbonitride were uniformly dispersed in the 18 percent-chromium steel. In this steel according to the present invention the matrix was ferrite as shown in Table 9, so it could eliminate the defects of the 18-8

50

Table 8

| Test items                                 | Test condition | Invented steel | SUH 33B |
|--------------------------------------------|----------------|----------------|---------|
| S-attacking rate (mg/cm <sup>2</sup> /hr)  | In 100% SO     | 800°C 0.05     | 0.03    |
|                                            | do.            | 900°C 0.17     | 0.25    |
| Oxidation rate (mg/cm <sup>2</sup> /hr)    | In the air     | 800°C 0.00     | 0.00    |
|                                            | do.            | 900°C 0.03     | 0.01    |
| Pb-attacking rate (mg/cm <sup>2</sup> /hr) | In PbO         | 915°C 950      | 780     |
|                                            | (initially)    |                |         |
|                                            | do.            | 915°C 185      | 440     |
|                                            | (finally)      |                |         |

Since the steel according to the present invention contained 10 percent by weight chromium, its usability covers a temperature range up to 900°C, and as the re-

stainless steel caused by its being an austenite steel, and at the same time it showed the extraordinarily excellent resistivity in the oxidation and the sulphur attack at a

65

temperature above 900°C. Accordingly, the present steel may be used, under some circumstances, as a superior and yet cheap heat-resisting stainless steel in place of a costly 18-8 stainless steel.

jected to the 100 percent sulphurous acid gas at 1,100°C:

less than 0.00001 mm

C. The corrosion rate against lead (loss in weight

Table 9

| Test item                                                        | Test condition                   | Invented steel  | 18-8 Stainless Steel                          |
|------------------------------------------------------------------|----------------------------------|-----------------|-----------------------------------------------|
| Intergranular corrosion cracking                                 | By JIS-4304                      | not recognized  | observed cracking in 3 pieces among 10 pieces |
| Coefficient of heat expansion<br>( $\times 10^{-6}$ )            | 25° – 600°C                      | 11.0            | 17.8                                          |
| V-attack resistance<br>(loss in weight-mg/cm <sup>2</sup> )      | In V <sub>2</sub> O <sub>5</sub> | 48              | 45                                            |
| Pb-attack resistance<br>(loss in weight-mg/cm <sup>2</sup> )     | In PbO                           | 915°C × 1 hr    | 1,000                                         |
| Oxidation resistance<br>(increase in weight-mg/cm <sup>2</sup> ) | In the air                       | 900°C × 10 hr   | 0.0                                           |
|                                                                  | do.                              | 1,000°C × 10 hr | 2.1                                           |
| S-attack resistance<br>(increase in weight-mg/cm <sup>2</sup> )  | In 100% SO                       | 800°C × 10 hr   | 0.5                                           |
|                                                                  | do.                              | 900°C × 10 hr   | 1.2                                           |
|                                                                  | do.                              | 1,000°C × 10 hr | 2.8                                           |
|                                                                  |                                  |                 | 146                                           |

## EXAMPLE 3

A thermal reactor for the exhaust of automobiles demands a heat-resisting steel which can stand the high temperature gas above 1,000°C, but the hitherto known heat-resisting steels have not met this desire in such points as the resistivity against sulphur etc. According to the present invention, a steel which can answer such a desire could be manufactured by dispersing about 5 percent by weight titanium carbonitride into the steel consisting mainly of, by weight, 25 percent chromium, 20 percent nickel and 2 percent molybdenum. The experimental results of the steel were as follows:

A. The thickness of the oxidation layer when the steel was repeatedly subjected to the heating and the sudden cooling cycle of 1,000°C × 1 hour in the air:

in the first cycle . . . . . 0.00038 mm  
in the respective subsequent cycle (on the average) . . . . . 0.00004 mm/cycle

B. The thickness of the sulphurated layer when sub-

20 when immersed in lead oxide at 915°C)

initially: 500 mg/cm<sup>2</sup>/hr  
subsequently: 150 mg/cm<sup>2</sup>/hr

D. The momentary tensile strength and elongation at 1,000°C:

14.3 kg/mm<sup>2</sup> and 64.0 percent, respectively.

What is claimed is:

30 1. A heat-resisting nickel-free steel consisting essentially of a uniform dispersion of 2 percent to 10 percent by weight of one or more carbonitrides selected from the group consisting of titanium, zirconium, niobium, tantalum, and vanadium carbonitrides, 1-30 percent by weight of chromium and 0.2 to 30 percent by weight of one or more elements selected from the group consisting of boron, silicon, molybdenum, manganese, copper and aluminum and the balance being iron and unavoidable impurities.

\* \* \* \* \*

45

50

55

60

65